

Jan. 7, 1969

V. MEKLER ET AL

3,420,656

PROCESS FOR FORMING HARD OXIDE PELLETS AND PRODUCT THEREOF

Filed Sept. 2, 1966

Sheet 1 of 3



Fig. 1.

INVENTORS

Valentine Mekler  
Morgan C. Sze  
Ward J. Bloomer  
William V. Bauer

BY *Marn & Jangarathis*  
ATTORNEYS

Jan. 7, 1969

V. MEKLER ET AL

3,420,656

PROCESS FOR FORMING HARD OXIDE PELLETS AND PRODUCT THEREOF

Filed Sept. 2, 1966

Sheet 2 of 3



Fig. 2.

Fig. 3.

INVENTORS  
Valentine Mekler  
Morgan C. Sze  
Ward J. Bloomer  
William V. Bauer

BY *Marn & Jangarathis*  
ATTORNEYS

Jan. 7, 1969

V. MEKLER ET AL

3,420,656

PROCESS FOR FORMING HARD OXIDE PELLETS AND PRODUCT THEREOF

Filed Sept. 2, 1966

Sheet 3 of 3



Fig. 4.

INVENTORS

Valentine Mekler  
Morgan C. Sze  
Ward J. Bloomer  
William V. Bauer

BY *Marn & Jangarathis*

ATTORNEYS

1

3,420,656

PROCESS FOR FORMING HARD OXIDE  
PELLETS AND PRODUCT THEREOF

Valentine Mekler, New York, and Morgan C. Sze, Garden City, N.Y., Ward J. Bloomer, Westfield, N.J., and William V. Bauer, New York, N.Y., assignors to The Lummus Company, New York, N.Y., a corporation of Delaware

Filed Sept. 2, 1966, Ser. No. 577,055

U.S. Cl. 75—5  
Int. Cl. C21b 1/10

20 Claims

## ABSTRACT OF THE DISCLOSURE

Finely divided iron ore is mixed with a fluid carbonaceous material and agglomerated into pellets at a temperature in the range of 400°–650° F. The fluid material should have a 5% boiling point of at least 650° F. The green pellets are coked at 700°–1000° F. to drive off volatile components, which are recovered, and form an evenly dispersed coke structure. The pellets are indurated and partially reduced at 1500°–2200° F. The resulting pellets are very strong, contain little or no free carbon, have less than 5% metallic iron, the balance being mainly FeO.

This invention relates generally to a process for agglomerating, hardening and partially reducing an oxide ore prior to its introduction into a metallurgical furnace. More specifically, the invention relates to the treatment of iron oxide ores, such as taconite fines, by agglomeration at 400°–500° F. using a heavy oil residue as binder, coking at 700–1000° F., and hardening and reducing at 1500°–2200° F., preferably below about 2100° F. The invention also relates to the pellets themselves, which are reduced about 15–40%, with some metallic iron and with little or no free carbon. Partial reduction per se is not the main objective of the invention, but it does provide the crushing strength necessary for blast furnace usage, and of course the reduction raises blast furnace efficiency.

As is well known in the art, pig iron is produced from iron ore, coke and limestone introduced into a blast furnace. At the point of entry of the air into the blast furnace, high temperatures are attained as a result of the exothermic heat of combustion of coke with air. The carbon monoxide formed by the incomplete combustion of coke and unburned coke reduce the iron oxide to iron. Impurities present in the ore and coke form a slag with the limestone. Molten pig iron and slag are periodically removed from the hearth of the blast furnace.

Since the blast furnace is a shaft furnace, it is necessary that the ore, coke and limestone be aggregates of fairly large particle size. The amount of fines in the charge materials should be minimized since fines can be blown out of the furnace as dust and can also plug up the shaft, thereby resulting in a high pressure drop. A number of factors are of importance in regard to the materials charged to the furnace. For example, since metallurgical coke is relatively expensive, it is obvious that the amount required per ton of product should be minimized. Furthermore, lower coke requirements reduce the amount of ash necessary to be slagged out, and thereby reduce the amount of limestone required to be introduced into the blast furnace, consequently resulting in higher furnace capacity and lower production cost per ton of product.

Recently, taconite ore—a low-grade iron oxide ore—has been increasingly mined as a result of decreasing supply of high grade ores. Beneficiation of taconite usually involves grinding the ore to form very small

2

particles of fines, followed by magnetic separation of iron values ( $Fe_3O_4$ ). The fines are agglomerated into pellets prior to charging the ore into a blast furnace. Agglomeration of the ore generally consists of pelletizing or briquetting the fines with the assistance of a binding agent, and then heating the resulting material to a high sintering temperature in the order of 2200–2400° F., to increase the strength of the pellets. In commercial pelletizing plants, bentonite clay and some solid carbonaceous fuel are added to the concentrate. The mixture is then passed through a balling drum (where the wet bentonite-concentrate mixture is made into balls of, for example,  $\frac{1}{4}$  to  $\frac{3}{4}$  " size); a vibrating feeder and a sintering machine wherein, at a temperature of approximately 2350° F., hardened pellets are produced. The pellets are thereafter cooled, screened and stored for shipment.

Briquetting differs from pelletizing only in that the binder-ore mixture is formed into shape by pressing rather than by balling, as for example in briquetting rolls, or by extrusion.

Several disadvantages characterize the present practice of pelletizing. High sintering temperatures are required to provide hardness and high strength to the pellets consequently using substantial quantities of fuel. Such pellets are not large aggregates and therefore high blast rates in the furnace cannot be used. This is especially so, since the size of the pellets is much smaller than the size of the coke and limestone used. The optimum size range of the pellets should be near the size range of the limestone and coke. Additionally, the use of an ash-containing carbonaceous fuel to supply the heat for agglomeration increases the amount of slag which has to be produced. Since the finished pellets are not reduced at all, they cannot effect any saving in metallurgical coke requirements. Highly reduced pellets are produced by various processes, all of which use solid carbonaceous fuels for reduction and for heat. The pellets have varying amounts of residual carbon. The ash content is inversely related to the quality—and cost—of the solid fuel.

Numerous procedures have been proposed to overcome disadvantages of the character indicated above. For example, it has been proposed to use a tar oil or a petroleum oil with an iron oxide concentrate, rather than a solid carbonaceous fuel, but strong, reduced pellets were not produced. It has also been proposed to use an asphalt with an oxide ore; however, even when temperatures of the order of 1500–1600° F. are used in forming a carbon-impregnated oxide ore aggregate, little physical strength is developed. A further proposal of prior workers was to initially mix the ore with tar at the mine site to render it non-dusting. At the steel mill, it was mixed with powdered coal and this mixture was briquetted and carbonized. Of course the coal addition brings back the ash problem noted above. Accordingly, while a number of such proposals have been made, there has been little or no success in providing oxide ore pellets having sufficient hardness to withstand the rigor of mechanical handling and thermal shock before and after being introduced to an agglomerating furnace. Nor has there been success in reducing the fuel requirements in preparing such agglomerates, or the ash content of the pellets.

It is an object of the present invention, therefor, to provide a process for forming oxide ore in pellet form of desired strength and hardness, of suitable size for efficient use in a metallurgical furnace, and of low ash content.

It is another object of the invention to form such pellets at relatively low temperatures and at an economical level of fuel consumption.

A further object is to provide partially reduced iron oxide ore in pellet form of said desired characteristics, whereby blast furnace coke requirements are reduced.

Another object of the invention is to provide iron oxide ore in pellet form containing low residual free carbon.

Still another object of the invention is to provide a process for forming oxide ore pellets utilizing inexpensive carbonaceous materials.

Yet another object of the invention is to provide a hard, partially reduced iron oxide pellet having the above-noted characteristics.

Various other objects and advantages of the invention will become clear from the following description of several embodiments thereof, and the novel features will be particularly pointed out in connection with the appended claims. The description will refer to the accompanying drawings, which are illustrative only and should not be interpreted in a limiting sense, and in which:

FIGURE 1 is a greatly simplified, pictorial flow sheet depicting the essential elements of the process as carried out in illustrative apparatus;

FIGURE 2 is a greatly simplified, schematic flow sheet depicting the solids flow in a second embodiment of the invention;

FIGURE 3 is a greatly simplified, schematic flow sheet depicting the solids flow and liquid recovery in an embodiment of the invention designed to product 3000 t.p.d. of product pellets; and

FIGURE 4 is a simplified, schematic flow sheet depicting gas and liquid flows for the embodiment illustrated in FIGURE 3.

While the description made herein of the invention is primarily directed to the treatment of iron oxide ores, it is to be understood that other oxides ores can be treated.

The foregoing objects are realized by a process comprising the following steps:

(a) Mixing the fine ore with a fluid carbonaceous material and agglomerating the mixture into pellets, all at a temperature of about 400°-500° F. These two steps are preferably carried out continuously in a suitable pelletizing machine so that the resulting pellets show a uniform cross-section of the ore and binder.

(b) Heating the green pellets to a temperature in the range of 700°-1000° F. to coke the heavy hydrocarbon binder, driving off volatile components and resulting in a pellet having coke evenly dispersed therein. Heating at this stage should be indirect to avoid combustion of the volatiles or dilution thereof with the heating gases.

(c) Further heating the pellet to a temperature in the range of 1500°-2200° F., during which heating the pellet is hardened and partially reduced.

Optionally, limestone or the like may be added during mixing, particularly if slag-formers are present in the ore, or if either the ore or the hydrocarbon contain sulfur or sulfur compounds.

The last heating should of course be carried out in a non-oxidizing atmosphere. Subsequent cooling of the pellets should also be conducted in the absence of air or oxidizing gases, until the pellets reach a temperature where reoxidation is no problem (below about 600° F.).

A variety of hydrocarbon materials may be employed in the process of the invention. Any heavy residual oil, vacuum residual oil, coal tar pitch or the like may generally be employed; it is desirable that the material have a Conradson Carbon content of at least 15% and preferably 20%, and have a 5% boiling point of at least 650° F. The term "5% boiling point" means that 95% of the residual oil boils above the specified temperature. It is further noted that a coal tar pitch would produce more coke and less distillate than the oils discussed hereinbelow and in the examples.

The pellets produced by the process will vary in composition depending on the amount of carbonaceous material added and the length of time at the various tempera-

tures. It is preferred, however, to produce a pellet reduced about 15-40% (25-35% preferred), in terms of total combined oxygen, in which there is some metallization and little or no free carbon. Such a pellet is characterized by a very high crushing strength and a fine porous structure which is eminently suitable for use in a blast furnace or other reduction device. In the case of pellets made from taconite or other high-grade concentrates, both the coke rate and fluxing required for reduction in the blast furnace are significantly reduced. The amount of metallic iron will not generally exceed about 5% when the pellets are intended for blast furnace usage, but it will be understood that by adjustment of oil addition and residence time, a sponge iron product can be produced. Preferably, the reduction is carried out so that the pellet, as discharged from the reducer, contains about 80% or more FeO, and, as noted above, little or no free carbon and some metallic iron. If cooling is very slow, it is possible that the FeO will disproportionate into Fe and Fe<sub>3</sub>O<sub>4</sub>, at least according to some prior workers. Under near equilibrium conditions, a metallic iron content of 20% may be achieved. However, under normal (non-oxidizing) gas cooling, which is quite rapid, the FeO structure is substantially retained. For this reason the pellet structure is characterized as it is "prior to cooling or after rapid cooling." Regardless of cooling rate, pellets of the preferred composition have an oxygen-to-iron (weight) ratio in the range of about 0.15 to 0.34.

In FIGURE 1 there is illustrated a very simple embodiment of the invention illustrating the essential steps thereof. Residual oil preheated so as to be flowable and ore from a bin are supplied to a rotating pelletizing drum. The oil and ore may be separately preheated to the preferred pelletizing temperature before they are charged, or the pelletizing drum may be provided with heating means. Oil is sprayed continuously on the ore, which agglomerates during its passage through the pelletizer. Any vapors evolved during this stage are combined with coker distillate for recovery of valuable constituents.

The pellets discharging from the pelletizing kiln pass through an intermediate hopper and are charged into the coking kiln, which is an indirectly fired travelling grate kiln. In this kiln, the pellets are heated to about 700°-1000° F. and vapors are driven off. The oil vapors are then passed to a recovery section from an outlet at one end. A seal hopper passes the coked pellets to the hardening and reducing kiln, which in this instance is a direct-fired, travelling grate kiln, where the pellets are heated to 1500°-2000° F. or higher. Removal of combustion gases is via a line in the charge end which leads to appropriate solids removal and heat recovery equipment (not shown). A travelling grate kiln is preferred for this service as the 1000° F. pellets discharged from the coker will probably not be hard enough to withstand handling in a rotary kiln.

The hardened pellets pass from the reducing kiln through another seal hopper to a pellet cooler, where their sensible heat is given up with the production of high-pressure steam. This pellet cooler is provided with inlets and outlets on the tube side for steam generation, inlets and outlets for supplying an inert or non-oxidizing atmosphere to the pellets, and an outlet for discharging cool pellets (<600° F.) to conveyor. The high pressure steam generated in this cooler may be conveniently utilized to preheat the oil prior to injection into the pelletizing kiln or to drive any rotating equipment.

In FIGURE 2 there is illustrated a more detailed embodiment of the invention. As noted above, the formation of green pellets is preferably carried out in a pelletizing drum and in this embodiment the ore and oil are preheated (not shown) and the drum itself is not heated. The fines, which are generally at least 70% minus 325 mesh, are conveyed to the pelletizing drum having been mixed with recycle dust and, if desired, limestone prior to

preheating. A preheated heavy oil is supplied to the drums in the same manner as illustrated in FIGURE 1. As shown in FIGURE 2, recycled solids come from a product screen and a green pellet screen, but it will be understood that solids will also be collected by cyclones or other equipment from various gas flows. Where appropriate, recycled material should be suitably crushed and ground before charging to the pelletizing drum.

The oil injection and pelletizing operation is carried out at 400° to 500° F. by preheating in order to secure a viscosity of the residue oil suitably low to provide an effective oil spray and to ensure that the oil intimately wets the charging ore and the accreting pellets to achieve uniform dispersion of the carbon for reduction.

The retention time of the pellets in the balling and mixing apparatus should be sufficient to permit the relatively slow growth of balls from an original minuscule size to an eventual 1/2, 3/4 or 1 to 1 1/2 inch size, as desired.

When discharged from the pelletizing drum, undersize may be screened. At this stage they have little mechanical strength and must be handled carefully. The green pellets are conveyed to an indirectly-fired travelling grate kiln similar to that shown in FIGURE 1 for coking. Of course, any device capable of indirect heating and in which the pellets are quiescent can be employed. Indirect heating is necessary so that the distillate can be recovered separately without combustion inside the kiln or dilution with combustion gases. Such indirect-heated furnaces are well known in the art. Oil distillate passing out of the kiln is sent to the recovery unit. The coking kiln is operated at a temperature which will distill essentially all volatile matter out of the pellets and thoroughly coke the remaining carbon. This is generally in the range of 750° to 1000° F., but in this embodiment a higher discharge temperature is desirable so that the pellets will be sufficiently hard to be subsequently treated in a direct-fired rotating kiln. A two-section kiln may be employed in this service. The cracked vapors begin to evolve in volume at about 750° F. and resemble in composition those secured in a conventional delayed coking operation. The non-condensable gaseous portion is rich in methane and hydrogen and, after recovery, is used in the fuel firing systems, as noted hereinbelow.

Since the reduction of  $Fe_2O_3$  to  $Fe_3O_4$  begins at about 850° F. and does not become appreciable until about 1100° F. is reached, reduction in the coker, even at the higher discharge temperature, is relatively minor; the major heat requirements are thus due to sensible heat duties and the endothermic cracking of hydrocarbons in the residual oil.

The distillate may be passed to a condenser where its sensible heat is recovered, and thence to a knock-out drum from which liquid and non-condensables are withdrawn separately or, it may flow directly to a fractionating tower, without being cooled, and processed as vapors from delayed coking drums are normally handled. In most instances a portion of the recovered distillate is used for fuel purposes, and appropriate local storage facilities (not shown) must be provided.

As noted above, the coked pellets should have sufficient mechanical strength to withstand subsequent handling and treatment by the time they leave the coking kiln. The coked pellets are transferred, while hot, to the charge end of the reducer kiln, where hardening and partial reduction takes place. A hopper seal wherein the pellets form a gas seal is preferred. This kiln is a direct-fired rotating kiln as shown, but may be an indirectly or directly fired tunnel kiln or other suitable device capable of maintaining temperatures in the desired 1500°-2100° F. range, particularly if the pellets are still "soft." As all of the reductant is contained in the pellets themselves, the kiln atmosphere need not be strongly reducing, but of course it should be non-oxidizing. This is readily accomplished by using a deficiency of air in the firing mechanism. Residence time in the reducer kiln will vary,

depending on degree of reduction desired and other factors, but about 1/2 to 2 hours is normal. When the reducer kiln is directly fired, by means of a burner located in the discharge end, it may be desirable to inject some additional air at one or more points upstream therefrom so that unburned fuel will be burned and the entire kiln maintained within the desired temperature range. This so-called "side air" injection is well known in the art, and is done by mounting a fan on the outside of the kiln shell and blowing air into the kiln interior through a stainless steel pipe. Alternatively a substantial portion of the combustion gases withdrawn from the charge end can be recycled to the burner end where they will mix with the combustion products and provide a more uniform temperature distribution.

After discharge from the reducer kiln, the pellets are cooled, still in a non-oxidizing atmosphere, to a temperature under 600° F. Below this temperature surface re-oxidation is not a problem, and further cooling is done with air in a second cooler. Such coolers are of conventional design.

The cooled pellets are then screened, with undersize being recycled to the pelletizing drum after appropriate grinding. Oversize pellets are ready for storage or shipment.

FIGURES 3 and 4 are considered in detail in Example II set forth hereinbelow, but it is of interest to compare them with FIGURES 1 and 2. FIGURES 3 and 4 relate to a plant designed to produce 3000 t.p.d. of pellets.

On this scale, it is economical to use a fluidized bed heater to initially heat the concentrate. Further, a separate pellet heater prior to the coker and a calcining stage thereafter are desirable, although in terms of actual processing units it may be desirable to make the pellet heating stage part of the pelletizer or coker, and locate the calcining stage at the end of the coking kiln or the charge end of the reducer kiln.

As shown in FIGURE 3, the liquid recovery section is illustrated as producing five separate fractions, as might be done in a single combination fractionating tower. A small stream may be withdrawn from the bottom of the tower and recycled directly to the pelletizer in order to recycle any ore fines contained in the coker vapors and trapped in the fractionator liquid streams. This is labeled as a "slurry" stream in the drawing, and is distinguished from the heavy oil stream, which is the highest-boiling wholly liquid stream that is withdrawn. The lightest fraction of gas (tower overhead), comprising noncondensables and hydrocarbons up to propane ( $C_3$ ), is shown as being used as fuel in the reducer along with the heavy oil stream; those skilled in the art will appreciate that these streams are utilized separately, the gaseous stream being burned with a substantial deficiency of air to insure maintenance of a reducing atmosphere.

In the embodiment of FIGURE 3, separate  $C_4$ -400° F. gasoline and distillate oil streams are withdrawn as by-products. As shown in Example II, the thermal economy of the process is such that a credit can be obtained from these upgraded products.

The gas and liquid flows for the embodiment of FIGURE 3 are shown in FIGURE 4. Briefly, incoming air is first preheated by indirect heat exchange against the exhaust gases from the ore preheater and the pellet heater. The air, at about 500° F., is further heated to about 1100° F. in a fired heater. The hot air is passed primarily to the reducer burner, with minor sidestreams being taken off for combustion in the muffles of the calciner and coker. Coker gas and heavy oil from the liquid recovery still are burned in the reducer kiln with the preheated air, and the major portion of the combustion gas is recycled for even temperature distribution (side air injection may be used for this purpose, or a combination of both methods is possible). The next combustion gas off-take from the reducer, at about 1865° F., is passed first through the calciner muffle and then through the coker muffle, with ad-

ditional air being added at each stage. Effluent from the coker muffle is at about 1410° F., and is used for heating (without further combustion) in the ore and recycle heaters and in the pellet heater, either in series or in parallel. The combined effluent, now at about 600° F. and still containing considerable carbon monoxide, which is combustible, is first used to preheat incoming air, and then, after further cooling to about 100° F. (where water vapor is condensed) it is used to cool finished pellets. The gas is heated to about 1700° F. during the latter operation by the pellets, and is then used as fuel in the air preheater, which produces steam as a byproduct. For the conditions set forth in Example II, stream production is 150,000 lb./hr.

Understanding of the invention will be facilitated by referring to the following specific examples. Example I presents detailed data on a small scale operation and Example II provides thermal and material balances for a plant producing three thousand tons per day of hardened, partially reduced pellets. Example III discusses the pellet composition and FIGURE 5.

#### EXAMPLE I

Eight-hundred pounds of commercially purchased taconite concentrate had the composition shown in Table I and sieve analysis shown in Table II.

Table I.—Chemical composition

| Concentrate:                   | Weight pct. |
|--------------------------------|-------------|
| Total Fe                       | 63.4        |
| Total O <sub>2</sub>           | 26.12       |
| Silica, as SiO <sub>2</sub>    | 8.33        |
| P                              | 0.02        |
| Ca (as CaO)                    | 0.77        |
| Al <sub>2</sub> O <sub>3</sub> | 0.26        |
| Mn                             | 0.19        |
| Mg (as MgO)                    | 0.42        |
| S                              | 0.003       |
| L.O.I.                         | 2.8         |

Table II.—Sieve analysis

| Tyler screen: | Percent |
|---------------|---------|
| +18           | 0.1     |
| +60           | 0.1     |
| +35           | 0.4     |
| +100          | 0.8     |
| +200          | 6.1     |
| +325          | 14.3    |
| -325 (fines)  | 78.2    |
|               | 100.0   |

The steps of the process were carried out in a batch kiln externally wound with heating cable and equipped to provide an inert (N<sub>2</sub>) atmosphere. Some pre-dried concentrate was charged and the kiln was preheated to 450° F. Nitrogen-atomized hot heavy-oil residue was sprayed in while the kiln was turning at 8 r.p.m., and additional concentrate was continuously added. The residual oil was a topped crude with an IBP of 700° F., and 14° API gravity and Saybolt Universal viscosity of 320 and 145 seconds at 210° F. and 250° F., respectively. Oil addition was controlled so that, in the finished (coked) pellet, there was 0.092 pound of coke per pound of Fe.

After the pellets attained a satisfactory size (100% plus 1/2 inch), rotation was stopped and the temperature was raised to and held at, successively, 750°, 800° and 865° F. levels. The oil distilled off largely at the 750° F. level.

The pellets were transferred, while hot, to a horizontal muffle furnace and heated successively to 1500° F. and 2000° F., again in a nitrogen atmosphere. Considerable weight loss resulted from calcination and oxide reduction.

After 3 hours at 2,000° F., the furnace was turned off

and the pellets were allowed to cool, the nitrogen atmosphere being retained to prevent reoxidation.

An assortment of the pellets was subjected to crushing strength tests and chemical analysis. All pellets tested of 1/2" to 5/8" size had crushing (i.e. compressive) strength in excess of 300 pounds, as compared to 200-250 pounds exhibited by clay-pelletized taconites. Chemical analysis is set forth in Table III.

Table III.—Pellet composition

|                                             | Weight pct. |
|---------------------------------------------|-------------|
| Fe (combined)                               | 68.99       |
| Fe (metallic)                               | 0.85        |
| O <sub>2</sub> (combined)                   | 20.70       |
| SiO <sub>2</sub> and others (by difference) | 9.46        |
| Total                                       | 100.00      |

Reduction was about 31%, and in this instance the pellet was 80.34% FeO and 9.35% Fe<sub>2</sub>O<sub>3</sub>.

#### EXAMPLE II

Commercial taconite ore of the composition shown in Table I of Example I is preheated to 400° F. and fed continuously into a rotary pelletizer, together with recycle fines. A petroleum residuum fraction having the properties shown in Table IV is preheated to 400° F. and sprayed continuously into the pelletizer.

Table IV.—Petroleum residuum fraction

|                      | API          |
|----------------------|--------------|
| Conradson carbon No. | percent 19.6 |

The resulting green pellets are fed continuously into a travelling grate kiln, wherein the pellet temperature is raised from 400° F. to 750° F. by direct contact with hot gases. In a subsequent section of this kiln the pellets are further heated to 1000° F. This high temperature portion of the kiln is partitioned from the low-temperature section so as to minimize gas flow or interchange between the two sections. In the high-temperature zone, coking of the pellet binder material takes place. The cracked vapors are passed to a fractionating tower from which the following streams are removed: Coker Gas (C<sub>3</sub>'s and lighter), Gasoline (C<sub>4</sub>'s to 400 E.P.), Light Distillate Oil (400° to 750° F. B.R.), and Heavy Distillate Oil (750° to 1100° F. B.R.). Alternatively, of course, the cracked vapors may be just cooled to condense and recover a wide boiling range distillate oil and a fuel gas. Any ore fines entrained by the coker gases are scrubbed in the bottom of the still and are removed as slurry with some of the still bottoms. This slurry is recycled to the pelletizer.

The coked pellets are fed to a second travelling grate kiln, known as the calciner, wherein the pellet temperature is increased from 1000° F. to 1600° F. The material is heated indirectly by radiation from an overhead muffle. The coke binder in the pellets is devolatilized, generating a so-called "coker gas" which is subsequently used as fuel. Some reduction of the iron oxides in the pellets takes place, generating CO and CO<sub>2</sub>.

The 1600° F. calcined pellets are quite strong and can withstand subsequent treatment in a rotary kiln without excessive decrepitation. The rotary kiln is called the reducer. Here the pellets are heated by direct radiation from products of combustion to 2000° F. The coke contained in the feed pellets is virtually completely reacted, resulting in the reduction of the iron oxides to lower oxides and a small amount of iron. This reduction achieves induction, so that the cooled product pellets exhibit a high crushing strength, usually exceeding 300 lbs.

The reduced and hardened pellets are introduced into the top of a shaft cooler. Here, cool (100° F.) inert gas, free of air or oxidizing gases, is passed counter-current to the descending pellets, cooling the latter to approximately 115° F.

The cooled pellets are screened and the sized product is conveyed to storage. The undersize material, about 2% of the total cooler output, is ground and recycled to the ore heater. The material flows, to produce 250,000 lb./hr. or 3,000 t.p.d. of product pellets, are shown in Table V.

The fuel economy of this process is demonstrated in the last column of Table V, which indicates residuum feed of 1.22 bbl. and liquid by-product (gasoline and distillate oil) recovery of 0.73 bbl. per short ton of product pellets. The actual fuel cost is further reduced by the differential in the per-barrel value of the upgraded liquid by-product as compared to the distressed residuum feed-stock.

The fuel economy results from the gas and liquid flow system, shown in FIG. 4. The coker gas and calciner gas are burned with a deficiency of air (preheated to 1100° F.). This is augmented with combustion of the heavy oil to release the energy required in the rotary kiln reducer. The effluent gas from the reducer is rich in CO, due to the CO content of the products of combustion (the gaseous fuels being burned with a deficiency of air), augmented by the CO generated by the ore reduction. An amount of the effluent gas may be recycled to the kiln inlet to lower the inlet gas temperature and achieve a fairly even temperature distribution in the kiln. This recirculation is, however, not always required.

The net reducer effluent gas, at about 1865° F., is introduced into the heating chamber of the travelling grate calciner. A little preheated air (1100° F.) is introduced into this gas to burn some of the contained CO as required by the heat balance.

The calciner effluent gas, at 1550° F., passes to the heating chamber of the coker. More preheated (1100° F.) air is introduced, burning a little more of the CO to maintain heat balance. The gas issues from the muffled heating chamber at about 1410° F. About 60% of this 1410° F. gas is then passed directly through the pellets on the travelling grate. Four passes are used to achieve counter-current heat exchange. This portion (60%) of the gas stream leaves the travelling grate kiln (pellet heater-calciner) at about 730° F.

The remainder (40%) of the 1410° F. gas leaving the coker muffled zone is passed through the ore and undersize recycle heater. This is a shallow-bed fluidized bed unit. The powder is heated to 400° F., and the gas issues at about 410° F.

Many variations of this processing scheme are possible: For example, the reducer could be a travelling grate kiln. The temperature levels can be varied considerably, for example, the calciner pellet discharge temperature could be set at 1700° F. instead of 1600° F. at 1700° F., significant reduction will occur. Also, instead of combining the pellet heater and coker functions in one travelling grate kiln, other combinations are quite possible.

The gas flow pattern can be modified to meet specific plan requirements. All of the 1410° F. gas from the coker muffle chamber can be passed through the pellet preheat zone, leaving at about 990° F. (instead of 730° F.); all or most of this gas can be passed through the ore and recycle heater. In some cases, it may be advantageous to spill some of the 1410° F. gas directly to the boiler-air preheater burner to improve temperature control and reduce cooling water requirements.

The following advantageous features of the general processing scheme should be noted: Although wide latitude in processing equipment is permissible, and desirable due to variations in ore, residuum, etc., the use of low-attrition devices (such as travelling grate kilns) up to a pellet temperature level of 1400° to 1800° F. insures low pellet degradation and low ore recycle requirements. Use of indirect heating in the 750° F. to about 1500°-1700° F. range insures fairly complete recovery of gaseous fuels and liquid by-products. Also, use of reducing atmosphere and relatively uniform temperature in the reducer permit relatively rapid reduction to proceed to the desired level. The desired action is further aided by the gradual and continuous release of CO (and equilibrium concentration of CO<sub>2</sub>) from the surface of the pellet bed, acting as a gas blanket to prevent excessive contact of the bed with the combustion gases above the bed.

The use of a relatively reducing gas as the cooling medium in the pellet cooler, combined with the relatively rapid heat transfer due to direct contact exchange, insures against pellet reoxidation. However, good heat recovery may be accomplished with suitable heat recovery equipment as shown in FIG. 1.

### EXAMPLE III

A pellet picked at random from those produced in Example I was sectioned, mounted and photomicrographed so as to display the microstructure resulting from the process of the invention.

TABLE V.—MATERIAL FLOWS, 3,000 T.P.D. PELLET PRODUCTION

|                              | Ore<br>Feed<br>(dry) | Resid. | Recycle<br>undersize<br>material | Green<br>pellets | Coked<br>pellets | Product<br>pellets | Coker and<br>calciner<br>cracked<br>gases | Fuel  | Liq. by-prods. |                | Flows in<br>bbl./ton<br>of prod.<br>pellets |
|------------------------------|----------------------|--------|----------------------------------|------------------|------------------|--------------------|-------------------------------------------|-------|----------------|----------------|---------------------------------------------|
|                              |                      |        |                                  |                  |                  |                    |                                           |       | Flow<br>rate   | Grav.<br>° API |                                             |
| Iron oxides                  | 246.8                |        | 22.7                             | 269.5            | 269.5            | 226.6              |                                           |       |                | 7.4            | 1,220                                       |
| SiO <sub>2</sub> , CaO, etc. | 23.4                 |        | 2.3                              | 25.7             | 25.7             | 23.4               |                                           |       |                |                |                                             |
| Residuum                     |                      | 54.4   |                                  | 54.4             |                  |                    |                                           |       |                |                |                                             |
| C <sub>3</sub> —             |                      |        |                                  |                  |                  |                    |                                           |       |                |                |                                             |
| C <sub>4</sub> to 400° E.P.  |                      |        |                                  |                  |                  |                    | 5.65                                      | 5.65  |                |                |                                             |
| Lt. distill                  |                      |        |                                  |                  |                  |                    | 9.75                                      |       |                | 58             | 300                                         |
| Hvy. distill                 |                      |        |                                  |                  |                  |                    | 10.95                                     |       | 10.95          | 16             | .262                                        |
| Coke                         |                      |        |                                  |                  |                  |                    | 12.95                                     | 4.45  | 8.50           | -8.5           | .169                                        |
| Total                        | 270.2                | 54.4   | 25.0                             | 349.6            | 312.9            | 250.0              | 39.30                                     | 10.10 | 29.20          |                |                                             |
| Ore/Pellet Anal:             |                      |        |                                  |                  |                  |                    |                                           |       |                |                |                                             |
| Fe, Wt. percent              | 64.7                 |        | 69.9                             | 55.0             | 61.4             | 69.9               |                                           |       |                |                |                                             |
| O/Fe, Wt. ratio              | .412                 |        | .296                             | .402             | .402             | .296               |                                           |       |                |                |                                             |
| Coke/Fe, Wt. ratio           |                      |        |                                  |                  |                  |                    | .091                                      |       |                |                |                                             |

NOTE.—All Flows in 1,000's of lbs./hr.

The cool gases (730° and 410° F.) are heat exchanged against cool air, then they are cooled with water to 100° F. The cooled gases, still reducing due to residual CO content, are passed counter-currently through the descending bed of pellets in the pellet cooler. The gases are thereby heated to about 1685° F.

The reheated gases are burned with additional air (cold) to consume the residual CO, and are used to preheat air to the desired level (1100° F.) and to generate plant steam.

A porous, essentially two-phase structure is present, the lesser phase being gangue materials and the majority of the structure being iron oxide. It is believed that the etching technique employed selectively removed metallic iron from the surface. Macroscopic examination revealed that the cross-section of the pellet was entirely uniform. With the method used it was not possible to distinguish between various iron oxide compositions.

It is to be understood that many other modifications can be made to the process illustrated in the drawings. For

example, the concentrate and oil can be milled at the 400°-500° F. temperature to form an even mixture, and then briquetted or extruded, while hot, in conventional equipment. The green briquettes are then treated in the same manner as the green pellets. Further, sufficient carbonaceous material can be added to bring about substantially complete metallization, with the production of sponge iron pellets suitable for melting and finishing, for example, in an electric furnace.

The preferred pellet composition, discussed hereinabove, is decidedly advantageous, however, for use in a blast furnace. For example, at a 30% reduction level the coke rate in a blast furnace can be 200 lb./ton of hot metal lower than for unreduced pellets. This drop in the coke rate allows the production rate of the furnace to be increased by about 20% at the same wind rate. The exact degree of reduction desired in any instance will depend on economic consideration.

Various other changes in the details, steps, materials and arrangements of parts, which have been herein described and illustrated in order to explain the nature of the invention, may be made by those skilled in the art, within the principle and scope of the invention as defined in the appended claims.

The present application is related to copending U.S. application Ser. No. 316,359, filed Oct. 15, 1963, now abandoned, and assigned to the same assignee.

What is claimed is:

1. A hardened, thermally treated, partially reduced iron-oxide bearing pellet which, prior to cooling or after 30 rapid cooling is characterized by a finely porous structure and consists essentially of:

at least about 70% FeO;

essentially no free carbon;

0-5% metallic iron;

balance higher iron oxides and impurities;

said pellet being chemically reduced about 15-40%.

2. The pellet as claimed in claim 1, wherein the compressive strength is at least 300 pounds, and size is about 1/2 to 1 1/2 inches in diameter.

3. A thermally treated, partially reduced iron-oxide bearing pellet which, prior to cooling or after rapid cooling, is characterized by a finely porous structure and a crushing strength of at least 300 pounds, a size of about 1/2 to 1 1/2 inches in diameter, and consists essentially of:

at least 70% FeO;

0-5% metallic iron;

0-5% CaO;

essentially no free carbon;

balance higher iron oxides and impurities;

said pellet being chemically reduced about 25-35%.

4. A hardened pellet consisting of:

0-20% metallic iron;

0-5% CaO;

essentially no free carbon;

balance iron oxides and impurities;

said pellet being characterized by an oxygen-to-iron weight ratio in the range of about 0.15 to 0.34, and having a finely porous structure and a crushing strength of at least 300 pounds.

5. The process for agglomerating and beneficiating an oxide ore comprising:

forming pellets by agglomerating said ore with a heavy hydrocarbon oil having a 5% boiling point of at least 650° F., said agglomeration being carried out at a lower but still elevated temperature where said oil is fluid;

heating the pellets thus formed to a temperature between said boiling point and the temperature where significant reduction of said ore begins to occur for a sufficient time to coke said oil and bake said pellets; and

further heating said pellets to reducing temperature, whereby said pellets are hardened and residual carbon therein effects reduction.

6. The process as claimed in claim 5, wherein said pelletizing is carried out at a temperature in the range of 400° to 650° F.

7. The process as claimed in claim 5, wherein said coking is carried out at a temperature in the range of 5700° to 1000° F.

8. The process as claimed in claim 5, wherein said reduction and hardening are carried out at a temperature in the range of 1500° to 2200° F. in a non-oxidizing atmosphere.

9. The process as claimed in claim 7, wherein said coking is carried out in an indirectly fired heater wherein said pellets are in a quiescent state, and additionally comprising recovering distilled volatiles driven off during said coking.

10. The process as claimed in claim 8, wherein said reduction and hardening are carried out in a direct-fired rotary kiln and said non-oxidizing atmosphere is provided by burning fuel with a deficiency of air.

11. The process as claimed in claim 5, wherein the quantity of said oil and said reduction are controlled to provide a finished pellet reduced about 15-40%, having 0-5% metallic iron, and essentially no free carbon.

12. The process for producing hardened, prereduced iron oxide pellets reduced about 15-40% comprising:

forming green pellets by mixing iron ore with a heavy hydrocarbon oil, said oil having a 5% boiling point in the range of about 650° to 1100° F., at a temperature in the range of about 400° to 500° F.; coking said green pellets by heating to a temperature in the range of about 700° to 1000° F. for a sufficient time to coke the heavy hydrocarbons and permit the cracked volatile constituents of said oil to be driven off;

hardening and reducing said pellets by heating to a temperature in the range of about 1500° to 2200° F. in a non-oxidizing atmosphere; and cooling the hardened and reduced pellets in a non-oxidizing atmosphere.

13. The process as claimed in claim 12, wherein said recovered volatiles are utilized to provide endothermic reaction heat.

14. The process as claimed in claim 12, wherein said ore is a taconite concentrate.

15. The process as claimed in claim 12, wherein said oil addition and said reduction are controlled to produce a pellet containing 0-5% metallic iron and essentially no free carbon.

16. The process as claimed in claim 13, wherein volatiles recovered from said coking are fractionated and separate fuel gas and fuel oil fractions are recovered; said fractions are burned with a deficiency of preheated air in said hardening and reducing step; combustion gases resulting from said hardening and reducing step are used to supply heat to said coking step, and to preheat said air and said iron ore; and the cooled combustion gases are used to cool said pellets.

17. The process as claimed in claim 16, wherein combustion gases used in said cooling step are burned with air, and resulting combustion gases are utilized to further preheat said air.

18. The process as claimed in claim 16, wherein said coked pellets are calcined at a temperature of 1000° to 1600° F. prior to reduction, heat therefor being supplied by combustion gases from said hardening and reducing step.

19. The process as claimed in claim 18, wherein additional preheated air is burned with said combustion gases in said coking and calcining steps.

20. The process as claimed in claim 12, wherein said ore and said oil are separately preheated to 400° to 500° F. prior to formation of said pellets.

**13****References Cited****UNITED STATES PATENTS**

2,812,249 11/1957 Culberson et al. ----- 75—4  
2,918,364 12/1959 Lesher ----- 75—4 5  
3,118,757 1/1964 Peras ----- 75—26  
3,264,092 8/1966 Ban ----- 75—3

**14**

3,341,322 9/1967 Bailey ----- 75—26  
3,351,459 11/1967 Mills ----- 75—4  
L. SEWAYNE RUTLEDGE, *Primary Examiner.*  
ERNEST L. WEISE, *Assistant Examiner.*  
U.S. CL. X.R.  
75—4, 5